

## UNITED STATES PATENT OFFICE

RENÉ CLAVEL, OF BASEL-AUGST, SWITZERLAND

## DYEING OF CELLULOSE DERIVATIVES

No Drawing. Application filed January 18, 1923, Serial No. 613,533, and in Great Britain July 28, 1922.

In previous processes for dyeing acetyl celluloses in artificial silk, film, or other form, with developer dyes in which the application of the bases or developers is effected at low, ordinary or only moderately raised temperatures, it is found, more especially for dyeing the acetyl cellulose goods black for example, that it is often necessary, in order to obtain a sufficiently deep, full shade, to repeat the base applying, diazotizing and developing treatment. Also the time of treatment with the base and developer baths had to be sufficiently prolonged for obtaining deep shades in order that even dyeing should be effected.

Long and repeated treatment of cellulose acetate artificial silk for example is liable to cause wooliness and weakening of the fibre, and moreover the duplicated treatments render the process more expensive.

I have now found that by employing relatively high temperatures, e. g. above about 60° C. and preferably about 70°-95° C. or more in applying the developer bath, or both base and developer baths, or combined base and developer baths, the dyeing of cellulose acetate in artificial silk or other form can be rapidly carried out, while preserving the fibre or material, and also while necessitating only small quantities of dyeing materials. At the same time the surprising discovery has been made that the spotting which was liable to occur, especially with blue and black, with slow development, does not take place with the higher temperatures. The process is preferably carried out with employment of basic media, that is to say easily hydrolyzable salts of strong bases or the free bases themselves (as for example sodium acetate or caustic soda lye) in a base bath, and of acids or acid salts (as for example hydrochloric acid, acetic acid or acid sodium phosphate and which substances are included under the term "acidic substance") in a developing bath. In order to preserve or protect very fine yarns owing to the increased tendency to swelling due to high temperatures I may also with advantage employ protective colloids, such as gelatines, gelatine

soaps, sulphonated fatty acid soaps or the like in the baths.

In applying the invention in cases where both base and developer are applied in the same bath, it will be understood that acids and free bases or hydrolyzable salts will not be employed together in the same bath. Any of these may be employed alone, according to the character of the dye bases and developers.

## Example 1. (For black)

To dye 1 kg. of cellulose acetate artificial silk black, 25 gr. dianisidine hydrochloride and 50 gr. sodium acetate are dissolved in 20 litres of water. The temperature on starting is 45° C. which after 10 minutes is raised to about 75°-95° C. After about 1/4 hour the goods are washed once with cold water. Then follows the second bath, the so-called nitrite bath, with employment of 5% sodium nitrite and 16% hydrochloric acid (20% strength), all calculated on the weight of the goods, after 30 minutes' treatment in this bath at usual low diazotizing temperature or at ordinary temperature the goods are washed with water and transferred to the developing bath (volume of bath 20 litres to 1 kilo of goods), containing

15 gr. sodium salt of beta-oxynaphthoic acid  
5 gr. phenol or cresol  
20 cc. acetic acid (80%)

Development is commenced at 60° C. and the temperature is raised to about 75°-95° C. Time of development about 10 minutes. The goods are then washed with soft water at 45° C., then soaped at 60° C. and subjected to a cold brightening and scrooping bath if scroop is required. The scrooping bath may consist for example of water, formic acid and an oil emulsion of olive oil and olive oil soap.

## Example 2. (For blue)

In a similar way to the above a fine blue (for example navy blue) can be dyed. 1 kg. of cellulose acetate artificial silk hanks is introduced on dye sticks into a wooden dye vat containing 20 to 25 litres of water and 8

55

60

65

70

75

80

85

90

95

100

gr. of dianisidine hydrochloride and 5 cc. concentrated caustic soda lye or the corresponding amount of sodium acetate. Such a small quantity of caustic soda has practically no saponifying effect on the cellulose acetate. The goods are turned in the bath for 10 minutes while raising the temperature progressively to 75°-97° C. The hanks are then washed with hard water and transferred to 10 the diazotizing bath containing—

10% sodium nitrite  
20% hydrochloric acid

all calculated on the weight of the goods, and 15 the goods are turned in this bath during about half an hour. The goods are then washed in one hard water and transferred to the developing bath consisting of—

20 litres water  
1 litre boiled-off liquor  
10 gr. sodium salt of beta-oxynaphthoic acid  
50 gr. acid sodium phosphate.

The goods are turned several times at 60° 25 C. in the bath which is raised to about 75°-97° C. After 10 minutes the goods are washed, soaped, again washed and subjected to a brightening and scooping bath.

It is understood that the present invention 30 may be applied generally in processes for dyeing acetyl celluloses with development dyes, in whatever order the base and developer are applied to the goods or the diazotization effected, and that it may even be applied 35 in cases where base and developer are employed in one and the same bath, as proposed for example in my previous U. S. application S. No. 592,602.

Soluble salts especially chlorides, such as 40 magnesium chloride, ammonium chloride, zinc chloride or tin chloride, may be employed in the base baths, developer baths or combined base and developer baths if desired.

What I claim and desire to secure by Letters Patent is:

1. In a process for dyeing cellulose acetate with azo development dyes, treating the material with the developer component at above 60° C.

50 2. In a process for dyeing cellulose acetate with azo development dyes, treating the material with the developer component at above 70° C.

3. In a process for dyeing cellulose acetate 55 with azo development dyes, treating the material with the developer component at between 70° C. and 95° C.

4. In a process for dyeing cellulose acetate with azo development dyes, treating the material with both the base component and the developer component at temperatures above 60° C.

5. In a process for dyeing cellulose acetate with azo development dyes, treating the material with both the base component and the

developer component at between 70° C. and 95° C.

6. In a process for dyeing cellulose acetate with azo development dyes, treating the material with the developer component at above 70° C. in the presence of a protective colloid.

7. In a process for dyeing cellulose acetate with azo development dyes, treating the material with the developer component at above 75° C. in the presence of an acidic substance.

8. In a process for dyeing cellulose acetate with azo development dyes, treating the material with the base component at above 70° C. in the presence of a quantity of a basic medium insufficient to saponify substantially the cellulose acetate, and treating the material with the developer component at above 70° C. in the presence of an acidic substance.

9. In a process for dyeing cellulose acetate 85 with azo development dyes, the step of treating the material with the developer component at between 70° C. and 95° C.

10. In a process for dyeing cellulose acetate with azo development dyes, treating the material with the developer component at between 70° C. and 95° C., in the presence of a protective colloid.

11. In a process for dyeing cellulose acetate with azo development dyes, treating the material with the base component at between 70° C. and 95° C. in the presence of a quantity of a basic medium insufficient to saponify substantially the cellulose acetate, and treating the material with the developer component at between 70° C. and 95° C., in the presence of an acidic substance.

In testimony whereof I have hereunto subscribed my name.

RENE CLAVEL. 105

110

115

120

125

130